

No. 807,028.

PATENTED DEC. 12, 1905.

P. L. T. HÉROULT.  
PROCESS OF OBTAINING SOUND INGOTS.  
APPLICATION FILED JUNE 14, 1905.

FIG. 1.



FIG. 2



INVENTOR:

Paul Louis Toussaint Héroult,

By Attorneys,

Arthur O. Fraser & Co.

WITNESSES:

Fred White  
Rene' Bruine

# UNITED STATES PATENT OFFICE.

PAUL LOUIS TOUSSAINT HÉROULT, OF LA PRAZ, FRANCE, ASSIGNOR TO  
SOCIÉTÉ ELECTRO METALLURGIQUE FRANÇAISE, OF FROGES, ISÈRE,  
FRANCE.

## PROCESS OF OBTAINING SOUND INGOTS.

No. 807,028.

Specification of Letters Patent.

Patented Dec. 12, 1905.

Application filed June 14, 1905. Serial No. 265,174.

*To all whom it may concern:*

Be it known that I, PAUL LOUIS TOUSSAINT HÉROULT, a citizen of the Republic of France, residing at La Praz, Savoie, France, have invented certain new and useful Improvements in the Process of Obtaining Sound Ingots, of which the following is a specification.

It is well understood that in the casting of ingots of steel there is a tendency to form pipes along the central axis of the ingot, due to the solidifying of the ingot first at the bottom and sides and the subsequent contraction of the soft central portion in an outward direction. Hydraulic and other presses have been employed to compress the ingots as they solidify in order to prevent the formation of these pipes. The process of this application is designed to replace such pressing-machines and accomplishes the same result by cooling the outside of the ingot while the center is soft, causing the shell to contract and fill up the spaces which would otherwise be left in the center by the outward contraction of the metal. The cooling of the shell produces a contraction which squeezes the internal liquid steel toward the top of the ingot, and if the cooling is continued a sufficiently long time—say until the interior has become solid—the ingot will be sound in all parts. The cooling should be effected with a certain degree of care—that is to say, not too fast. The rapidity will be readily determined by a practical workman. The cooling may be effected by any suitable cooling fluid, such as a stream of water or a blast of cold air or gas. For example, any one of the following methods may be used: The sides of the mold may be raised, leaving the ingot standing on its base, and streams of water may then be applied on it, commencing at the bottom. The mold being removed, water may be run into the pit in which the ingot is usually cast, the depth of water being gradually increased. The ingot may be bodily lifted off its base and lowered into a bath of water.

The accompanying drawings illustrate the method first above described.

50 Figure 1 is a central section through a partly-cooled ingot in its mold. Fig. 2 is an elevation of the same ingot with the mold sides removed.

The ingot hardens at the bottom and sides

gradually toward the center, the irregular lines A indicating roughly the successive zones of solidification. When a sufficiently thick solid shell has formed to enable the ingot to stand alone, the interior being still substantially fluid, the mold sides B are lifted and jets of water played upon the ingot C from hose-nozzles D or the like, commencing at the base and working slowly up to the top. The cooling of the solid shell causes it to contract and to squeeze the fluid central portion so as to take up the contraction of such fluid portion, which would cause it to spread outward and form central pipes—that is to say, the inward contraction of the shell counteracts the outward contraction of the fluid central portion. By commencing at the bottom and when the interior of the ingot is very fluid the inward contraction of the shell will be greater than the outer contraction of the central fluid portion, and the latter may be squeezed upward. It is not proposed to continue the cooling operation after the central portion of the ingot has hardened so as to be practically beyond the possibility of contraction, but only to apply the cooling action at such a rate and to such an extent as will counteract the tendency of the central portion to form pipes or voids as it changes from a liquid to a solid state.

Though I have described with great particularity of detail certain embodiments of the invention, yet it is not to be understood therefrom that the invention is limited to the specific methods described. Modifications may be made by those skilled in the art without departure from the invention.

What I claim is—

The process of making sound ingots which consists in running the metal into a mold, permitting the ingot to harden sufficiently to form a solid shell while the interior is still substantially fluid, removing the mold, and applying a cooling fluid to the shell of the ingot to cause it to contract upon the central portion so as to prevent the formation of pipes in said central portion.

In witness whereof I have hereunto signed my name in the presence of two subscribing witnesses.

PAUL LOUIS TOUSSAINT HÉROULT.  
Witnesses:

DOMINGO A. USINA,  
FRED WHITE.